

# UNITED STATES PATENT OFFICE.

CARL AUER VON WELSBACH, OF VIENNA, AUSTRIA-HUNGARY, ASSIGNOR TO WELSBACH LIGHT COMPANY, OF GLOUCESTER CITY, NEW JERSEY, A CORPORATION OF NEW JERSEY.

## MANUFACTURE OF ELECTRIC FILAMENT.

1,109,886.

Specification of Letters Patent.

Patented Sept. 8, 1914.

No Drawing.

Application filed August 9, 1898. Serial No. 688,203.

To all whom it may concern:

Be it known that I, Dr. CARL AUER VON WELSBACH, a subject of the Emperor of Austria-Hungary, residing at Vienna, Austria-Hungary, have invented or discovered a new and useful Improvement in the Manufacture of Electric Filaments, of which the following is a specification.

The object of my invention is to produce 10 a filament substantially of osmium; another object is to provide a method of obtaining such a filament, and to this end to cover a platinum or other suitable wire with a coherent compact layer of osmium or an alloy 15 thereof of sufficient thickness of a homogeneous character and of requisite flexibility.

In the practice of my invention I produce upon a platinum or suitable wire a number of superposed layers of osmium or a compound 20 thereof. Subsequently the platinum or other wire is caused to form an alloy with the coating containing osmium. Afterward the platinum or other material of the wire is volatilized in whole or in part leaving a 25 filament containing osmium or osmium alloyed with the metal of the wire. Such a filament is somewhat pliable, is homogeneous and well adapted for use in electric incandescent lamps.

30 I have obtained good results in practice by the use of a platinum wire and I will describe my invention in connection therewith.

I prepare a diluted osmium compound in the form of a solution rendered, if necessary, a little more consistent by the addition 35 of finely divided osmium; or another solid osmium compound like sulfid or tetra-hydroxid may be used. I coat the platinum wire with such solution either by means of 40 a brush or other appropriate implement, or by passing the wire through the liquid. The wire is repeatedly passed through the liquid and heated to the drying point between each immersion or application until a 45 coating of the desired thickness is obtained. It may be remarked that it is best that each layer should be thin, so that the described operation of supplying each separate coat and then heating it must be repeated many 50 times in order to make the filament sufficiently thick. Although it may be accomplished with one sufficiently uniform coating application and of a drying heat. By thus depositing the osmium coating slowly 55 and uniformly the osmium filament finally

formed does not present bulges upon its outside. The unfinished filament is then exposed to the action of an atmosphere of reducing gases, and by the electric current gradually heated to above the temperature 60 at which platinum volatilizes. During this operation an alloy of platinum and osmium is formed and then the platinum is driven off from the alloy leaving only small traces 65 of the same and the filament becomes somewhat elastic and resembles platinum in color. A brittle alloy of osmium and platinum may result from the above described operation, but such an alloy lacks perfect 70 homogeneity. However, by gradually increasing the heat to which the filament is subjected by the passage through it of an electric current to the required temperature, the platinum of the alloy may be almost 75 completely volatilized without fusing the alloy itself while at the same time the described characteristics of the finished filament are insured. It is of importance that a sufficiently thick and uniform coating be obtained before the wire is subjected to the 80 final gradual application of the electric current up to the production of a temperature at which the core wire will volatilize. In lieu of platinum other metals may be used 85 provided they are sufficiently ductile and resist temperatures to which the filament is exposed in the course of its preparation, as well as other conditions to which the filament is subjected in the course of its manufacture. 93

As an example of the reducing gas to which reference has been made I may refer to gas obtained from the center of a Bunsen tube which is ignited at its air inlets which contains hydrogen, carbon-monoxid 95 and hydro-carbons, and which gas also contains water vapor.

One purpose of the application of heat between each application of the described coating is to reduce the coating to the metallic state, that is, in the present instance to osmium. Instead of supplying osmium or osmium compound in the form of a solution, as has been referred to, a very thin platinum wire may be covered or treated as described with a semi-liquid consisting of finely divided osmium or osmium compounds or of a mixture thereof with a small quantity of sugar or of another organic binding material and water or of another suitable fluid 110

which will form a kind of emulsion of the components. Ruthenium and rhodium either in whole or part or with osmium or its compounds may be used.

5. It will be understood that, in the method claims herein, I intend to include by the expressions "coatings containing osmium" and "coating containing osmium," a coating or coatings wherein osmium appears in any 10 of the specific forms described, *i. e.*, either in the form of a compound, or in the metallic form, or as a mixture thereof.

Having thus described my invention, what I claim is:

15. 1. The herein-described process of making filaments for electric incandescent lamps, which consists in repeatedly applying successive coatings containing osmium to a wire and subjecting the same to the action of a 20 drying heat between each coating, and then subjecting the coated wire to the action of an electric current in a protective atmosphere oxidizing as to any carbon present in the coating, until it is raised to a temperature 25 higher than the volatilizing temperature of its core; substantially as set forth.

2. The herein-described process of making filaments for electric lamps, which consists in repeatedly applying coatings containing osmium to a wire and subjecting the same to the action of heat between each coating, and finally exposing the coated wire in 30 a protective atmosphere oxidizing as to any carbon present in the coating, to a gradually 35 increasing temperature which finally is greater than the volatilizing temperature of the core; substantially as set forth.

3. The herein-described process of making filaments for electric lamps, which consists in applying coatings containing osmium 40 to a platinum wire and finally subjecting the coated wire to the action of an electric current in a protective atmosphere oxidizing as to any carbon present in the coating, up

to a temperature beyond the volatilizing 45 temperature of the platinum; substantially as set forth.

4. The herein-described process of making filaments for incandescent lamps, which consists in applying a coating containing 50 osmium to a wire, then subjecting the same to a drying heat and then to a gradually increasing electric current in a protective atmosphere oxidizing as to any carbon present in the coating, until the temperature of the 55 wire core exceeds its temperature of volatilization; substantially as set forth.

5. The herein described process of making metallic filaments for incandescent lamps, consisting in coating a wire core with a coating containing a metal having a point of fusion above the volatilizing point of the wire core, then subjecting the same to a drying heat and then to the action of the electric current, in the presence of a reducing 60 gas, until sufficient heat has been developed to volatilize the wire core and leave the metallic particles in a cemented or coherent condition; substantially as set forth. 65

6. The herein described process of making 70 metallic filaments for incandescent lamps, consisting in coating a wire core with a coating containing a metal having a point of fusion above the volatilizing point of the wire core, subjecting the same to a drying 75 heat and then to the action of the electric current, in the presence of the gas obtained from a Bunsen tube ignited at its air inlets, until sufficient heat has been developed to volatilize the wire core and leave the metallic particles in a cemented or coherent 80 condition; substantially as described.

Signed this 27th day of July 1898.

DR. CARL AUER VON WELSBACK.

Witnesses:

LUDWIG HAILINGER,  
ADOLF GALLIA.